

Patented July 2, 1929.

1,719,056

# UNITED STATES PATENT OFFICE.

WILLIAM GRENVILLE HORSCH, OF CORAOPOLIS, PENNSYLVANIA, ASSIGNOR TO VULCAN DETINNING COMPANY, OF SEWAREN, NEW JERSEY, A CORPORATION OF NEW JERSEY.

## RECOVERY OF ZINC.

No Drawing.

Application filed December 2, 1926. Serial No. 152,305.

This invention relates to the recovery of zinc from materials containing zinc and iron, and has for its object the provision of an improved method of recovering zinc from such materials. More particularly, the object of the invention is to provide an improved method of recovering zinc from galvanized iron, zinc dross and similar zinc and iron bearing materials.

10 The invention contemplates a substantially complete separation of the zinc from the iron in zinc and iron bearing materials, so that the iron remains in condition to be readily utilized for remelting. The zinc is preferably recovered in the form of an intermediate zinc oxide product, of a high degree of purity, which is readily converted into commercial products such as zinc chloride, zinc sulfate, etc.

15 In accordance with the invention, the zinc and iron bearing material is subjected to the action of an appropriate solvent that dissolves zinc but not iron and which enters the metastable condition as the zinc concentration increases. A solution of an alkali metal zincate containing an excess of alkali is a suitable solvent for this purpose. The presence of an oxidizing agent, such as an alkali metal nitrate, promotes the solution 20 of the zinc. The resulting pregnant solution is appropriately treated for the recovery of a zinc-bearing product therefrom.

In the preferred practice of the invention, the separation of the zinc from the iron is brought about by means of an alkaline sodium zincate solution of the proper absolute and relative concentrations of zinc and free sodium hydroxide. Thus, the concentration of total sodium hydroxide may lie within the 25 range of 200 to 400 grams per liter, while the zinc concentration, which is relatively low at the start, rises as solution or stripping progresses to from 100 to 200 grams per liter. An excess of sodium hydroxide should be 30 present in this solution; in other words, the solution is always alkaline. The recovery of the zinc in the form of a zinc oxide product from the resulting charged or pregnant solution by appropriate means leaves the alkaline sodium zincate solution in a regenerated condition for the treatment of fresh zinc and iron-bearing material.

The chemistry involved in the process may be outlined as follows: A solution of sodium hydroxide of a particular concentration will

dissolve a perfectly definite amount of zinc oxide, resulting in a certain definite zinc concentration. Such a solution, which has dissolved all of the zinc oxide that it will take up, is saturated with respect to zinc oxide, but not with respect to metallic zinc. In fact, the solution, after saturation with zinc oxide, is still capable of dissolving considerable zinc from the metallic state.

I have found, however, that solutions which have thus taken up zinc from the metallic state in excess of the equilibrium concentration corresponding to the solubility of zinc oxide exist in a metastable state. Such metastable solutions gradually deposit zinc oxide on standing until the zinc concentration falls to the equilibrium value. This attainment of equilibrium is extremely slow at room temperatures, requiring several months. At boiling temperature, however, the equilibrium concentration is attained in a few minutes. In view of investigations made at room temperatures and at boiling temperature, it is estimated by extrapolation that at relatively low temperatures, say zero degrees to 10° C., metallic zinc will be dissolved until practically all of the free sodium hydroxide has been used up as indicated by the equation:



85

In carrying out the invention, in accordance with my preferred practice, the zinc and iron-bearing material is treated with a cold solution (preferably below about 30° 90 C.) of sodium zincate containing an excess of sodium hydroxide. The addition of sodium nitrate to the solution increases the speed of the reaction. After the solution has dissolved as much zinc as it can safely take 95 up, the resulting pregnant solution is transferred to a recovery apparatus of appropriate construction, where the solution is heated with or without the addition of water. This heating causes zinc oxide to be precipitated 100 and free sodium hydroxide to be liberated. If water was added to the pregnant solution prior to or during heating, the solution resulting from the precipitation step must be reconcentrated by evaporation. After reconcentration, this solution is then ready for the treatment of further zinc and iron-bearing material.

When water is used for dilution of the pregnant solution, the reconcentrated solu- 110

tion is found to contain less zinc than corresponds to the solubility of zinc oxide. Such a solution may be heated without causing the precipitation of zinc oxide. 5 Advantage may be taken of this fact by utilizing the freshly reconcentrated hot solution as the final solution or stage of a counter-current system. In this way, more nearly complete removal of the zinc from 10 the zinc and iron-bearing material is effected. After the zinc has approached, but not reached, a concentration corresponding to the solubility of zinc oxide therein, the solution may be cooled down and employed 15 as the first stage in the counter-current solution system, building up now with zinc to the metastable condition.

Several alternative methods of recovering the zinc from the pregnant solution may be 20 practiced. For example, the pregnant solution may be refrigerated to cause the separation therefrom of crystals of sodium zincate. These crystals may be hydrolyzed readily to form zinc oxide and free sodium 25 hydroxide. Again, the pregnant solution may be treated with an appropriate agent such as sodium carbonate, carbon dioxide, hydrogen sulphide or the like, to effect precipitation of zinc oxide or other zinc 30 compounds.

The zinc oxide product obtained by the aforementioned procedures is of a high degree of purity containing only slight amounts of iron, but this zinc oxide product 35 does not possess the requisite physical properties to make it generally marketable. This zinc oxide product, however, is an intermediate product of considerable value because of its ready conversion into marketable compounds of zinc, such as zinc chloride, zinc sulfate, commercial zinc oxide, etc., thus making for diversification of output.

The production of high grade commercial zinc chloride or zinc sulfate necessitates calcining the zinc oxide product prior to its treatment with acid for solution of the zinc. The calcination takes place in an oxidizing or non-reducing atmosphere at about 50 a red heat. Such calcination destroys organic matter arising from grease and dirt on the original zinc and iron-bearing material, and also converts any ferrous iron present to the ferric condition. The latter 55 is essential to the precipitation of iron by zinc oxide. Sodium chlorate or other oxidizing agents will also bring about this oxidation of the ferrous iron and destroy most organic matter, but the use of these 60 reagents is generally objectionable on account of the impurities introduced.

The present invention is of particular advantage in the recovery of zinc from scrap and waste products, such as galvanized iron 65 scrap and zinc dross. In the treatment of

such scrap and waste products, it is of advantage to preliminarily wash the material in hot dilute caustic or carbonate solution to prevent grease or other organic matter from entering the stripping solution. 70

I claim:

1. The process of recovering zinc from materials containing zinc and iron which comprises subjecting the material to the action of a solvent that dissolves zinc but not iron to form a metastable solution as the zinc concentration increases, and recovering a zinc-bearing product from the resulting solution. 75

2. The process of recovering zinc from materials containing zinc and iron which comprises subjecting the material to the action of an alkaline solvent containing a zincate to form a metastable solution, and recovering a zinc-bearing product from the resulting solution. 80

3. The process of recovering zinc from materials containing zinc and iron which comprises subjecting the material to the action of an alkaline solvent containing sodium zincate to form a metastable solution, and recovering a zinc-bearing product from the resulting solution. 85

4. The process of recovering zinc from materials containing zinc and iron which comprises subjecting the material in the presence of an alkali metal nitrate to the action of a solution of an alkali metal zincate, and recovering a zinc-bearing product 90 from the resulting solution. 95

5. The process of recovering zinc from materials containing zinc and iron which comprises subjecting the material in the presence of an alkali metal nitrate to the action of a cold solution of an alkali metal zincate containing an excess of alkali, and treating the resulting solution for the precipitation of a zinc oxide product therefrom. 100

6. The process of recovering zinc from materials containing zinc and iron which comprises subjecting the material in the presence of an alkali metal nitrate to the action of a cold solution of an alkali metal zincate containing an excess of alkali, and heating the resulting solution and thereby 110 precipitating a zinc oxide product therefrom.

7. The process of recovering zinc from materials containing zinc and iron which comprises subjecting the material in the presence of an alkali metal nitrate to the action of a cold solvent solution of an alkali metal zincate containing an excess of alkali, and treating the resulting solution for the precipitation of a zinc oxide product therefrom and simultaneously regenerating said 120 solvent solution.

8. The process of recovering zinc from materials containing zinc and iron which comprises subjecting the material in the presence of an alkali metal nitrate to the 125

action of a cold solvent solution of an alkali metal zincate containing an excess of alkali, heating the resulting pregnant solution and thereby precipitating a zinc oxide product 5 therefrom, and calcining said zinc oxide product.

9. The process of recovering zinc from materials containing zinc and iron which comprises subjecting the material to a two-  
10 stage solution treatment in the first stage of which the solvent is a cold solution of an alkali metal zincate and in the second stage of which the solvent is a hot solution of an alkali metal zincate, heating the pregnant  
15 solution resulting from the first solution stage and thereby precipitating zinc oxide and regenerating the solvent solution, utilizing said hot regenerated solution as the solvent in the second solution stage, cooling the  
20 pregnant solution from the second solution

stage, and utilizing said cooled solution as the solvent in the first solution stage.

10. The process of recovering zinc from materials containing zinc and iron which comprises subjecting the material in two 25 stages to the action of solvent solutions of an alkali metal zincate containing an excess of alkali, the solvent solution in the first stage being cold and in the second stage being hot, heating the pregnant solution resulting from the first solution stage and thereby precipitating zinc oxide and regenerating a solvent solution, utilizing said regenerated solution while hot as the solvent in the second solution stage, cooling the 30 pregnant solution from the second solution stage, and utilizing said cooled solution as the solvent in the first solution stage.

In testimony whereof I affix my signature.  
WILLIAM GRENVILLE HORSCH.